

(Model.)

S. D. CASTLE.  
BASE BALL.

No. 281,238.

Patented July 17, 1883.



Witnesses  
S. S. Thompson  
W. W. Mortimer

Inventor

Sam'l. D. Castle,  
by Worcester Smith  
Atty's

# UNITED STATES PATENT OFFICE.

SAMUEL D. CASTLE, OF BRIDGEPORT, CONNECTICUT.

## BASE-BALL.

SPECIFICATION forming part of Letters Patent No. 281,238, dated July 17, 1883.

Application filed May 23, 1883. (Model.)

*To all whom it may concern:*

Be it known that I, SAMUEL D. CASTLE, a citizen of the United States, residing at Bridgeport, in the county of Fairfield and State of Connecticut, have invented certain new and useful Improvements in Base-Balls; and I do hereby declare the following to be a full, clear, and exact description of the invention, such as will enable others skilled in the art to which it appertains to make and use the same.

My invention relates to balls, and has for its object to produce a ball which shall be more durable than any ball now in use, shall be free from seams and imperfections, and which may be produced at a much less expense than any ball now upon the market.

With these ends in view my invention consists in a ball having a seamless gutta-percha cover.

20 My invention also consists in a ball having a cover of gutta-percha deposited thereon by dipping in a liquid solution of that material until the cover shall have attained the requisite thickness; and, finally, my invention consists in the process of covering balls by dipping them in a liquid solution of gutta-percha, dissolved in bisulphide of carbon.

For the purpose of enabling those skilled in the art to which my invention appertains to understand and apply it, I will proceed to describe the same, referring to the accompanying drawing, forming a part of this specification.

The drawing is a sectional view of an ordinary ball.

35 A represents the body of the ball, which may be made of any material, and B represents the cover. This cover is of gutta-percha and is without seam or break of any kind. I ordinarily use drip gutta-percha; but the refined article may be used, if preferred. The gutta-percha may be dissolved in any well-known solvent; but bisulphide of carbon is preferred, as it is quite cheap and its action is perfect. 40 The strength of the solvent is not a matter of importance. Having prepared the solution, the ball is grasped by a pair of grippers and dipped in the solution. The ball may be dipped any number of times. The weaker the solution the more dippings are required. It is

better always to dip the ball more than once. The completed cover need not be more than from one thirty-second to one-sixteenth of an inch in thickness. It is not a matter of the slightest importance of what material the ball 55 is made, as I have found my cover to work equally well upon all kinds of balls now in the market. In covering, the first dipping should be for some seconds, in order that the gutta-percha may sink into the interstices of the 60 ball. After the first dipping I usually let the ball stand for a few moments, in order that the gutta-percha may harden. It is then rolled for a short time, to smooth down any irregularities on the surface. This rolling, however, is not an essential feature, and I often omit to roll them when the balls are smooth and round. After the cover has been dipped the requisite number of times—that is to say, when the deposit of gutta-percha has become 65 sufficiently thick—the balls are allowed to stand for ten or twelve hours, when they become sufficiently hard for use. I have usually found from three to five dippings sufficient. Before putting them upon the market I prefer 70 to remove the gloss by a slight rubbing with fine sand-paper. This leaves the cover slightly rough, and gives it a leathery appearance. Should any imperfections in the gutta-percha be deposited upon the ball, or should the ball 75 be uneven after the final dipping, the irregularities may be removed by sand-paper; or, if preferred, the balls may be placed in a lathe and dressed with sand-paper, or in any other manner. After the balls are dressed down 80 they may be dipped in a dye and given any desired color.

I have found by actual use that these covers are not affected in the slightest by any changes in the weather. They do not crack or chip, 85 and withstand an almost unlimited amount of hard batting.

Having thus described my invention, what I claim to be new, and desire to secure by Letters Patent, is—

1. As an article of manufacture, a ball having a seamless cover of gutta-percha.
2. A ball having a cover of gutta-percha deposited thereon by dipping in a solution of said material.

95

100

3. A ball having a cover of gutta-percha deposited thereon by dipping in a solution of said material, and colored by dipping the completed ball in a dye solution.
- 5 4. The process of covering balls, which consists in dipping the ball in a solution of gutta-percha dissolved in bisulphide of carbon.

In testimony whereof I affix my signature in presence of two witnesses.

SAMUEL D. CASTLE.

Witnesses:

A. M. WOOSTER,  
GEORGE A. KINNER.